

## 1

3,233,985

**METHOD FOR THE PRODUCTION OF AN IMPROVED METAL/CERAMIC MATERIAL AND ARTICLES**

Paul Kraft and Josef Schloemer, Reinbek, Bezirk Hamburg, Germany, assignors to Wurttembergische Metallwarenfabrik, Geislingen an der Steige, Germany.  
No Drawing. Filed July 6, 1962, Ser. No. 208,089.  
Claims priority, application Germany, July 10, 1961.

J 20,217

4 Claims. (Cl. 29—191.2)

The invention relates to a process for the production of an improved metal/ceramic material and articles made therefrom, and relates especially to ceramic materials and shaped articles which contain a metal skeleton.

It has been known for some time that metal fibres, which are usually obtained by cutting from metal wires, filaments and the like, can be felted together and, as felts, can be sintered to shaped articles (so-called fibre-metallurgy). It is also known that a porous skeleton-like metal molded article so produced is able to serve as a reinforcing structure for, for example, pure magnesium. Following on from this it was hoped that it would be possible to build the metal fibres into ceramic compositions as reinforcement. Experiments showed, however, that when the usual iron or steel wool was used together with a fluid suspension of ceramic powders in liquids (so-called "slip"), such as those with aluminum oxide as the main constituent no metal/ceramic articles with useful properties could be obtained. This is probably caused in part by the formation of iron-aluminum oxide spinels, which have very bad mechanical properties and, in comparison with aluminum oxide, a very low-eutectic melting point of  $1310^{\circ}$  C.

It has now been found that these disadvantages can be removed and a metal/ceramic material with good mechanical, thermal and chemical properties can be produced by first subjecting metal wool, especially steel wool, to a diffusion treatment with a relatively inert metal thereby improving the heat- and corrosion-resisting qualities, then annealing and, after cooling, treating with suitable ceramic, oxide/ceramic or metal/ceramic slips, drying and if desired compressing the drying mass while being in a leather-hard condition.

It is also possible to stratify the steel wool, before the diffusion treatment, in the form of single fibres, and to press it to any desired shape. After this the diffusion treatment is effected.

It has been found expedient to use the steel wool in fibre thicknesses of a maximum of 0.6 mm., preferably less than 0.1 mm. As a general principle the thickness of the fibres should be the smallest possible, i.e. the lower limits for the thickness of the fibres are set by the process of preparation for the steel wool. It has further been found that the carbon content of the steel may be varied within relatively wide limits. In the process according to the invention a steel wool with more than 0.1% of carbon may be used; in some cases even with more than 1% of carbon. The steel wool, the diffusion metal, the diffusion process and the oxide/ceramic mixture must be chosen with respect to composition so that everything is successively synchronised. These are the usual tasks for the technicians in the metal and ceramic fields.

For some uses it may be expedient to provide the surface of the shaped article produced, after drying, with an additional coating of a carbide ceramic slip, preferably by dipping or spraying. The metal/ceramic so obtained consists according to the invention of a metallic and a ceramic phase, which are interconnected together at the phase boundaries in the form of interlocking net-

## 2

works, while the metallic phase may consist of homogeneously chromed steel wool. The ceramic phase, just as the steel wool skeleton, is a network and only the subsequently applied surface layer is a continuous layer.

5 This material according to the invention possesses excellent mechanical, technological, thermal, oxidation-resisting and corrosion-resisting properties, which is to be attributed to the fact that the homogeneously chromed steel wool possesses a good adhesion to ceramic compositions, especially to aluminum oxide.

10 The good adhesion between chromed steel wool and ceramic according to the invention may possibly be attributed to a mechanism similar to that known from combination materials using aluminum oxide and chromium powder, which materials show a transition phase of chromium oxide-aluminum oxide spinel (ruby) formed at the phase boundaries between the chromium metal and aluminum oxide.

15 The relative amounts of ceramic material (aluminum oxide) and chromed steel wool to be used depend upon the purpose of use. The greater the properties of chromed steel wool, the higher is the toughness and impact strength of the finished material. As a rule parts by volume of aluminum oxide and chromed steel wool in the proportion of 1:1 are aimed at.

20 In addition, the density of the material according to the invention can be adjusted to the intended purpose and vary with the preparation. When the metal fibres, which may be cut to certain suitable length, e.g. to 5-50 mm., are chromed and annealed and the resultant fibres, now homogeneously enriched with chromium, are mixed with the slip and then sintered in a furnace, a comparatively dense material with a bulk density between 4.0 g./cc. and 5.0 g./cc. results. Higher bulk densities are obtained when this material is compressed as, after the pre-drying, it is in the so-called leather-hard state, or when, before the chromising, the steel wool is sintered to skeleton-like bodies, the latter are then chromed and annealed, and the bodies so treated are saturated with the slip and again are compressed when being in the leather-hard state, after having been dried. This process is especially suitable for the production of parts of complex shape, especially turbine blades.

25 If steel wool with a relatively high carbon content is used, then on chromising, fairly large amounts of chromium carbide are formed in the chromium alloy. Since carbides have a more or less ceramic-like character, the binding of such a steel wool in the ceramic base material is still better. For this reason according to the present invention the chromising of steel wool with a higher carbon content is preferred, which is in contrast to the recommendations in the literature, according to which the carbon content in every case is said to be not allowed to exceed 0.1%.

30 Such a material may be converted into ceramic cutting discs with relatively good cutting properties by coating with a so-called "cermet"-material, which possesses especially good cutting properties. The said cermet-material means a powder combination of ceramics and refractory metal oxides with other metals and alloys, especially such as aluminum oxide-chromium combinations, and is described by Blackburn, A. R. and Shevlin, T. S. in "Progress Report on Fabrication and Physical Properties of Chromium-Aluminum Oxide Cermets,"

35 Ohio State University, April 1949 (Report N. 53). The coating of cermet-material is applied to the dry steel wool/ceramic body by dipping or spraying and post-sintering the whole. Upon use as a cutting tool, the steel wool/ceramic body part plays the role of providing the strength, whereas the coating part provides the cutting properties.

A thin coating layer of a few tenths of a millimetre of the cermet is sufficient. These cutting discs cannot of course be subsequently sharpened, but must be used as "expendable discs."

The shaped articles produced by the process according to the present invention, on account of their great strength and good heat conductivity, are particularly advantageous for use as material for machine parts and cutting discs.

The following examples are for the purpose of illustration, only, without limiting the present invention in scope.

*Example 1*

Steel wool in the form of many single fibres with a fibre thickness less than 0.01 mm. and an average fibre width of about 0.1 mm. was prepared by chipping off from a special steel wire with the following analysis: 0.13% C, 1.06% Mn, 0.042% P, 0.009% S, 0.05% Cr and traces of Si. The length of the fibres was variable and extended up to a few metres. The steel wool so obtained was packed loosely in a suitable chromising vessel with pieces of chromium and subjected to a chromium diffusion treatment with gaseous hydrogen chloride for 3 hours at 1100° C. The steel wool was then annealed at 1300° C. for 5 hours under a reducing atmosphere, whereby a homogeneous distribution of the chromium over the whole fibrous cross-section of the steel wool is obtained.

After cooling, a steel wool resulted which had an average chromium content of about 30%. The steel wool so obtained was again split up into separate fibres and mixed with a composition consisting of 95%  $\text{Al}_2\text{O}_3$  and 5% of kaolin. This mixture was compressed in a mould at a pressure of 5 tons per  $\text{cm}^2$  and sintered in vacuo at 1550° C. for 1 hour. After cooling, a shaped body was obtained which consisted of ceramic and 50% by volume of chromised steel wool and which had a good heat conductivity as well as comparatively high strength.

*Example 2*

The metal wool was prepared from steel wire as described in Example 1, and the fibres arranged in a directed form in separate layers and at various angles to one another. The fibres so arranged were first compressed in a rectangular mould with a pressure of 0.5 ton/ $\text{cm}^2$ . A mutual interlocking of the separate fibres took place, so that after the pressing the pressed body already had a shape corresponding somewhat to the final form.

The preliminary moulded body was now chromised by the process described in Example 1. The chromising temperature however was 1200° C. and the chromising time 2 hours. After this period, the current of hydrogen chloride was stopped and the chromising vessel purged with hydrogen, the temperature being maintained for a further 3 hours. A homogeneously chromised metal frame-work, alloyed all the way through, was obtained which, after cooling was steeped in the ceramic composition mentioned as the slip in Example 1. After drying, while in the leather-hard state, the body obtained was further compressed at 2 tons/ $\text{cm}^2$ , and then further dried at 95° C. for 10 hours. After this, sintering in vacuo for 1 hour at 1550° C. was carried out. A metal/ceramic body resulted which, with regard to its physical, technological and chemical properties, was even somewhat superior to the body mentioned in Example 1.

*Example 3*

A shaped body was first moulded from steel wool as in

Example 2 and subjected to sintering for 1 hour at 1350° C. in a current of hydrogen. The individual fibres are welded together by this treatment, and the steel wool skeleton possesses a high strength with very great porosity. The steel wool framework was then chromised for 3 hours at 1100° C., as described in Examples 1 and 2. A subsequent equalising annealing at 1300° C. in a current of hydrogen brought about homogenisation of the content of chromium. The annealing period was about 5 hours. The skeletal body so obtained was saturated in vacuo with a ceramic slip according to Example 1, dried in air at 95° C. and then compressed at 2 tons/ $\text{cm}^2$  while in the leather-hard condition.

The final sintering took place at 1550° C. for 1 hour in a high vacuum. The metal-ceramic body so obtained had very good properties.

*Example 4*

A shaped body was prepared by the process given in Example 2 and chromised, but the carbon content of the steel wool amounted to 1.2%. This shaped body was saturated with the composition mentioned in Examples 1 and 2 and dried. It was then dipped into a fluid carbide/ceramic slip composition and the excess carbide/ceramic suspension was removed by draining off, so that only a layer of about 0.2 mm. thickness remained adhering thereto. This shaped body obtained further plastic properties through the suspension liquid adsorbed and was then dried while in the leather-hard state and compressed with 6 tons/ $\text{cm}^2$  in a steel mould. The sintering was effected in vacuo at 1700° C. for a period of 1 hour. The shaped body so obtained, after careful grinding with a diamond whetstone, could be used for machining on a lathe.

We claim:

1. A method of producing a body of metal fibers in a ceramic matrix, comprising contacting a body of ferrous metal fibers with metallic chromium and heating the body of metal fibers to diffuse the chromium throughout the thickness of the fibers, thereafter impregnating the body of fibers with a ceramic slip, and thereafter sintering the ceramic of the impregnated body.
2. A method as claimed in claim 1, in which the ceramic is principally aluminum oxide.
3. A method as claimed in claim 1, in which the ferrous metal has a carbon content in excess of 0.1%.
4. A metal fiber ceramic impregnated material comprising a metallic phase in the form of an interlocking network of homogeneously chromised steel wool of a thickness up to about 0.6 mm., the network being impregnated with a fused ceramic material which adheres firmly to the steel wool.

References Cited by the Examiner

UNITED STATES PATENTS

- |           |         |         |       |          |
|-----------|---------|---------|-------|----------|
| 3,068,556 | 12/1962 | Kramer  | ----- | 29—420 X |
| 3,153,279 | 10/1964 | Chessin | ----- | 29—419 X |

FOREIGN PATENTS

- |         |         |            |
|---------|---------|------------|
| 210,927 | 10/1957 | Australia. |
|---------|---------|------------|

OTHER REFERENCES

- "Fiber Metals," Materials and Methods, Metcalfe et al., November 1955, pp. 96-98.

WHITMORE A. WILTZ, Primary Examiner.